

(No Model.)

E. H. & A. H. COWLES.

2 Sheets—Sheet 1.

PROCESS OF SMELTING ORES BY THE ELECTRIC CURRENT.

No. 319,795.

Patented June 9, 1885.

FIG. 1.



FIG. 2.



WITNESSES

C. J. Bell  
O. H. Clark

INVENTORS

Eugene H. Cowles  
Alfred H. Cowles  
By Paine & Ward,

Attorneys

(No Model.)

E. H. & A. H. COWLES.

2 Sheets—Sheet 2.

PROCESS OF SMELTING ORES BY THE ELECTRIC CURRENT.

No. 319,795.

Patented June 9, 1885.

FIG. 3.



WITNESSES

C. J. Belts.  
O. A. Clark.

INVENTORS

Eugene H. Cowles  
and Alfred H. Cowles,  
By Paine & Ladd,  
Attorneys.

# UNITED STATES PATENT OFFICE.

EUGENE H. COWLES AND ALFRED H. COWLES, OF CLEVELAND, OHIO, AS  
SIGNORS, BY DIRECT AND MESNE ASSIGNMENTS, OF FOUR-TENTHS TO  
EDWIN COWLES AND CHARLES F. MABERY, BOTH OF SAME PLACE.

## PROCESS OF SMELTING ORES BY THE ELECTRIC CURRENT.

SPECIFICATION forming part of Letters Patent No. 319,795, dated June 9, 1885.

Application filed December 24, 1884. (No model.)

*To all whom it may concern:*

Be it known that we, EUGENE H. COWLES and ALFRED H. COWLES, citizens of the United States, residing at Cleveland, in the county of Cuyahoga and State of Ohio, have invented 5 certain new and useful Improvements in Processes for Smelting Ores by the Electric Current; and we do hereby declare the following to be a full, clear, and exact description of the 10 invention, such as will enable others skilled in the art to which it appertains to make and use the same, reference being had to the accompanying drawings, and to letters or figures of reference marked thereon, which form a 15 part of this specification.

The present invention relates to the class of smelting-furnaces which employ an electric current solely as a source of heat. Heretofore it has been attempted to reduce ores and perform metallurgical operations by means of an 20 electric arc, the material to be treated being brought within the field of the arc or passed or fed through it; but numerous experiments have demonstrated that the arc system is not 25 adapted for long and continuous operations on a scale of any considerable magnitude. The difficulties attending the regulation of the arc and the preservation of a constant resistance are very great, and the heat generated, though 30 intense, is localized and difficult to control.

The object of this invention is to provide a process by which electricity can be practically employed for metallurgical operations, and for this purpose to secure a distribution of the 35 intense heat which it is well known electricity is capable of generating over a large area or through a large mass in such a manner that a high temperature can be sustained for a long time and controlled.

To this end the invention consists, essentially, in the use for metallurgical purposes of a body of granular material of high resistance or low conductivity interposed within the circuit in such a manner as to form a continuous 45 and unbroken part of the same, which granular body by reason of its resistance is made incandescent and generates all the heat required. The ore or light material to be reduced—as, for example, the hydrated oxide of 50 aluminium, alum, chloride of sodium, oxide of

calcium, or sulphate of strontium—is usually mixed with the body of granular resistance material, and is thus brought directly in contact with the heat at the points of generation at the same time the heat is distributed through 55 the mass of granular material, being generated by the resistance of all the granules, and is not localized at one point or along a single line. The material best adapted for this purpose is electric-light carbon, as it possesses the necessary amount of electrical resistance, and is capable of enduring any known degree of heat when protected from oxygen without disintegrating or fusing; but crystalline silicon or other equivalent of carbon can be employed 60 for the same purpose. This is pulverized or granulated, the degree of granulation depending upon the size of the furnace. Coarse granulated carbon works better than finely-pulverized carbon and gives more even results. The 70 electrical energy is more evenly distributed, and the current cannot so readily form a path of highest temperature and consequently of least resistance through the mass along which the entire current or the bulk of the current 75 can pass; but the scope of this invention is not limited by the degree of granulation, as that may vary with the conditions of the case, and with a large furnace and a powerful current the size of the carbon particles may pass 80 beyond what is ordinarily understood by the term "granular" and be, in fact, pieces of carbon of considerable size. Still the resistance body is ordinarily composed of grains or pieces 85 proximately equal in size, in order to secure an even distribution of the electrical energy.

The operation must necessarily be conducted within an air-tight chamber or in a non-oxidizing atmosphere, as otherwise the carbon will be consumed and act as fuel. The 90 carbon acts as a deoxidizing agent for the ore or metalliferous material treated, and to this extent it is consumed, but otherwise than from this cause it remains unimpaired.

We will illustrate and describe a zinc-furnace embodying our invention, from which the application of the same to the reduction or smelting of other kinds of ores will be readily understood, especially of aluminium, silicium, magnesium, boron, and other rare 95

metals, which are not reducible by the smelting processes heretofore known.

Figure 1 is a vertical longitudinal section through the center of a zinc-retort of a form similar to those used in the Belgian furnaces, and Fig. 2 is a front view of the same.

This retort consists of a cylinder, A, made of silica or other non-conducting material, suitably embedded in a body, B, of powdered charcoal, mineral wool, or of some other material which is not a good conductor of heat. The rear end of the retort-cylinder is closed by means of a carbon-plate, C, which plate forms the positive electrode, and with this plate the positive wire of the electric circuit is connected. The outer end of the retort is closed by means of an inverted graphite-crucible, D, to which the negative wire of the electric circuit is attached. This graphite crucible serves as a plug for closing the end of the retort. It also forms a condensing-chamber for the zinc-fumes, and it also constitutes the negative electrode. The term "electrode" is used in this case as designating the terminals of the circuit proper, or that portion of it which acts simply as an electrical conductor, and not with the intention of indicating the ends of a line between which there is no circuit-connection. The circuit between the electrodes, so called, is continuous, being established by means of and through the body of broken carbon. The mouth of the crucible is closed with a luting of clay or otherwise, and the opening d, made in the upper side of the crucible, near its extremity, comes entirely within the retort and forms a passage for the zinc-fumes from the retort-chamber into the condensing-chamber. The pipe E serves as a vent for the condensing-chamber. The zinc ore is mixed with the pulverized or granular carbon and the retort charged nearly full through the front end with the mixture, the plug D being removed for this purpose. A small space is left at the top, as shown. After the plug has been inserted and the joint properly suited the electric circuit is closed and the current allowed to pass through the retort, traversing its entire length through the body of mixed ore and carbon. The carbon constituents of the mass become incandescent, generating a very high degree of heat, and being in direct contact with the ore the latter is rapidly and effectually reduced and distilled.

The heat evolved distills the zinc, and the zinc-fumes are condensed in the condensing-chamber precisely as in the present method of zinc-making, with this important exception, that aside from the reaction produced by heating carbon in the presence of zinc oxide the electric current in passing through the zinc oxide has a decomposing and disintegrating action upon it, not unlike the effect produced by an electric current in a solution. This action accelerates the distillation and promotes economy in the process.

It will be observed that the intimate mixture of incandescent carbon and ore affords the most effective utilization of all the heat evolved. None of it is lost by transmission through any intervening bodies or spaces. Moreover, the maximum degree of heat generated by the furnace is within the ore body, and the retort and furnace receive only the heat which is transmitted outward from the ore and carbon contained within; consequently the retort or the furnace is not subjected to the highest degree of heat, as is the case in the Belgian method of zinc-smelting, and the life-time of a retort is thus materially increased. It is proposed to use a number of these retorts in the same circuit, in series or multiple arc, as desired.

We have found in practice that a mixture of about one part of carbon with one and a half parts of zinc ore, by weight, gives most satisfactory results with the particular ore which we have treated; but the proportions to be used will depend upon the character of the ore and the degree of heat required to reduce it, and the degree of heat evolved will be determined by the resistance or conductivity of the mass and the strength of the current employed.

Fig. 3 illustrates an improved form of furnace operating in the same manner as the one just described.

The furnace or retort chamber F has an inclined floor, sloping from both ends down to a discharge-hole, f, through which the metal and slag or residue can be withdrawn. G G' are the electrode-plates forming the ends of the furnace-chamber, connected, respectively, with the electric wires. H is the condenser, and I I are hoppers for charging the furnace, several being provided, to distribute the charge evenly along the chamber. The hoppers I and the discharge-opening f are closed with fire-clay plugs. This furnace admits of the use of heavy walls and solid permanent construction, and also a prolonged heat. A nice regulation of the resistance of the charge is secured by means of the several feed-hoppers, an additional amount being fed in when resistance is too high, and a portion of the charge being withdrawn through the bottom when the resistance is too low.

In the reduction of an ore composed of a non-volatile metal, or a metal which is not volatilized at the heat generated in the furnace, the metal remains in the furnace mixed with the carbon filling the interstices between the grains, while the gases produced pass off. In the reduction of rare metals, where a pure product is desired, it is necessary to use a pure carbon, or a carbon free from iron or other foreign ingredient, otherwise the iron or other substance will go into the product.

We do not in this application make any claim to the furnace or apparatus herein described, as that is reserved for the subject-matter of a separate application; and we are aware that an electric current has been em-

ployed in the reduction of fused ores, and we do not claim the same, broadly, but

What we do claim as our invention, and desire to secure by Letters Patent, is—

- 5 1. The method of generating heat for metallurgical operations herein described, which consists in passing an electric current through a body of broken or pulverized resistance material that forms a continuous part of the electric circuit, the ore to be treated by the process being brought into contact with the broken or pulverized resistance material, whereby the heat is generated by the resistance of the broken or pulverized body throughout its mass, and the operation can be performed solely by means of electrical energy.
- 10 2. The method of smelting or reducing ores or metalliferous compounds herein described, which consists in subjecting the ore in the presence of carbon to the action of heat generated by passing an electric current through a body of broken or pulverized resistance material that forms a continuous part of the electric circuit, the ore being in contact with the broken or pulverized resistance material, whereby the ore is reduced by the combined action of the carbon and of the heat generated solely by the resistance of the broken or pulverized body throughout its mass.
- 15 3. The method of smelting or reducing ores or metalliferous compounds herein described, which consists in pulverizing the ore and mix-
- 20 ing with it pulverized or broken carbon or like material, then introducing the mixed ore and carbon within an electric circuit, of which it forms a continuous part, the said circuit being established through the carbon constituents of the mass, whereby the heat is generated by the electrical resistance of the carbon throughout the mass, and the operation can be performed entirely by means of the carbon reagent and the electrical energy.
- 25 4. The method of smelting or reducing ores or metalliferous compounds herein described, which consists in subjecting the ore in the presence of a reducing agent to the action of heat generated by passing an electric current through a body of broken or pulverized resistance material that forms a continuous part of the electric circuit, the ore being in contact with the broken or pulverized resistance material, whereby the ore is reduced by the combined action of the reducing agent and of the heat generated solely by the resistance of the broken or pulverized body throughout its mass.
- 30 In testimony whereof we affix our signatures in presence of two witnesses.

EUGENE H. COWLES.  
ALFRED H. COWLES.

Witnesses:

JOHN C. COVERT,  
C. A. WHITNEY.